

June 6, 1933.

A. A. F. M. SEIGLE

1,913,061

LIQUID FUEL

Filed Dec. 12, 1923



Patented June 6, 1933

1,913,061

# UNITED STATES PATENT OFFICE

ADOLPHE ANTOINE FRANÇOIS MARIUS SEIGLE, OF PARIS, FRANCE

## LIQUID FUEL

Application filed December 12, 1923, Serial No. 680,059, and in France May 19, 1923.

The invention has for its object, as a new industrial product, a liquid fuel which is essentially composed of carbon and hydrogen, but may accessorially if not accidentally, contain a small proportion of oxygen and traces of sulphur.

In fact, the invention relates to a new liquid which is very inflammable, although relatively not very light, and which can be industrially extracted in considerable proportions from the crude oils of petroleum or shale, fuel oils, gas oils and analogous substances of a petroliferous or shaly nature.

Hereunder are stated the main characteristic features which clearly differentiate the new hydrocarbon product of a very inflammable nature from those of the same class which are at present known in the industry and trade of petrols, gasolines, various liquid fuels etc.

Moreover a process of manufacture of the said product will be also hereinafter described, but solely by way of example.

One physical feature of the product according to the invention consists in the very abnormal concurrence of the following facts: the ignition point of the new product is somewhat below that of the usual gasoline extracted from petroleum, while possessing a density greater than that of the said gasoline, and a like calorific and thermodynamic efficiency.

Further characteristic features of a purely chemical nature are successively mentioned below; the new product has the same percentage composition of hydrogen and carbon as the non-inflammable and more or less heavy oils, and even viscous oils, from which it was extracted, and which, omitting their percentage of oxygen, sulphur etc., contain as a rule from 88 to 89 parts by weight of carbon for 12 to 11 parts of hydrogen, whilst the analogous composition of the standard gasoline is from 85 to 86 parts of carbon by weight for 15 to 14 parts of hydrogen, and this whatever may be the origin and percentage composition of the crude or heavy petroleums from which the said standard gasoline has been extracted.

In short, the aggregate of light hydrocar-

bons composing the product according to the invention is isomeric with the aggregate of the original heavy hydrocarbons, whilst (as is known) the hydrocarbons composing the standard gasolines obtained by cracking or by a mere distillation are, on the whole, the homologues of their original hydrocarbons, due to the increase in hydrogen or the diminution in carbon of the percentage composition of the latter.

Furthermore, the hydrocarbons composing the product according to the invention are mainly non-saturated hydrocarbons, whilst most of the homologous hydrocarbons entering into the composition of the standard gasolines are saturated hydrocarbons.

A direct consequence of this latter feature is that the new product is much more sensitive to the action of certain chemical agents than the gasolines of the standard type. For instance the sulphuric acid partially converts the new product into sulpho-conjugated derivatives or various sulphonated products whose colour varies from a bright red to a greenish brown and having strong odours revealing the presence of ketone derivatives such as menthone, eucalyptol etc.

On the contrary, chloride of calcium only forms a feeble precipitate which can be readily separated from the liquid thus purified and freed from colour, and whose ether-like odour is of a very characteristic nature.

The new product can always be recognized by its odour which remains very peculiar when it is in the crude state that is to say when it is discharged from the apparatus, as well as when it has been treated by one or another reagent.

This fact is all the more characteristic as it is constant, even when the origin of the crude or heavy petroleums or shale oils used as raw material is changed.

A further difference between the new product and the standard gasolines extracted from petroleum resides in that these latter are, as is well known, insoluble in the methyl ethyl, amyl alcohols, unless an auxiliary or solvent suitable substance, such as ether, be used, whereas the new liquid fuel is di-

rectly very soluble in all said alcohols, and in all proportions, if the alcohols are absolute, and as far as 80 to 85 percent of fuel in the industrial alcohols. Further, such alcoholic solutions are entirely stable, and remain liquid at a temperature of  $-35^{\circ}$  C.

The above-mentioned characteristics clearly differentiate the product according to the invention from the other light and inflammable hydrocarbons obtained from petroleum of shale, which are already known, and now will be given the principal characteristic features which differentiate the same from the equally light and inflammable hydrocarbon extracted from the coal-peat or lignite-tar, and which is usually sold under the denomination of "benzol".

1. When treated with nitric acid, the fractional parts of the new product which distil between 80 and 90° C., do not furnish nitro-benzine, whereas the same fractional parts of benzol will furnish it in abundance. In other words, this means that the improved fuel contains substantially no hydrocarbons of the aromatic series.

2. The new product in the crude state has a density of 0,735 to 0,780, according to the nature of the raw material from which it has been extracted, whilst refined benzol has a density of about 0,870 to 0,890.

3. A somewhat intensive cooling to  $-30^{\circ}$  or  $-35^{\circ}$  C. has no effect upon the new product, whereas benzol becomes frozen throughout the mass at  $-4^{\circ}$  C.

35 4. Leaving out of account its small proportion of oxygen, sulphur etc., the elementary composition of the new product is, as has been above said, from 88 to 89 parts by weight of carbon for 12-11 parts of hydrogen, whereas the average composition of benzol is 92 parts by weight of carbon for 8 parts of hydrogen.

Having thus explained the main chemical, physical and other characteristic features which differentiate the new hydrocarbon product of very inflammable nature according to the invention, from those of the same kind at present known in the industry and trade of petrols, gasolines, etc. I will now so describe by way of example one of the processes which can be used for the industrial manufacture of this new product.

In the appended drawing showing diagrammatically an installation for carrying out the said process into effect.

Fig. 1 is a general view, and Fig. 2 is a perspective view on a larger scale of a detail.

According to the herein described process any one of the raw materials above specified; 60 crude petroleum or shale oils, fuel oils, gas oils etc. . . may be used, but in order to facilitate the comprehension of the following process, the latter will be applied to the treatment of crude petroleum, wherefrom 65 the water and the usual gasoline have been

preliminarily extracted, and whose density at 15° C. is 0.897, its ignition point (in an open vessel) being 80° C. If such crude petroleum is treated by fractional distillation, no vapour is given off up to 140° C.; up to 200° C., 5 per cent is vaporized; up to 300° C., 33 per cent is vaporized; up to 350° C., 85 per cent is vaporized and the residue consists of 15 per cent of dry tar.

In a vaporization apparatus or boiler *v* 75  
suitably heated by a combustible of any kind,  
the oil is introduced in a continuous manner  
after having been preliminarily heated to  
200° C., as will be further explained; this  
petroleum is raised in the boiler to its tem-  
perature of maximum vaporization i. e.,  
350° C. and the hydrocarbon vapours thus  
generated are then brought to the bottom of  
a heating retort *A* of the type described in  
my copending U. S. Patent application Se-  
rial No. 607,902, filed December 19, 1922. 80 85

These vapours enter through the pipe *a*, according to the arrow 1, and at a pressure substantially equal to the atmosphere pressure, into the bottom of the worm retort A (Fig. 1), circulate upwardly by their natural ascension in the annular part *b* divided by the discs *c* (Figs. 1 and 2), and during this upward circulation they are caused to flow through metallic chips or turnings laid upon said discs.

This method of circulation affords a gradual and systematic superheating of the vapours of oil or heavy hydrocarbons to a determined and easily adjustable temperature, without risk of an abrupt decomposition, such as takes place in cracking apparatus; the metallic chips which these vapours are caused to meet with upon the whole of their path will on the one hand regulate the temperature and on the other hand will exercise a catalytic action upon these hydrocarbons.

The metallic fragments used are the waste from machine work upon pieces of iron, nickel, copper and other usual metals, and they are laid upon the annular discs *c* so that the temperatures assumed by these fragments when in contact with the central heating tube *t* shall correspond to the temperatures necessary for a suitable catalytic action.

In order to increase the combined effects of heat and catalysis and to ensure an effective stirring of the hydrocarbon molecules, the circulation of the latter is alternately reversed, according to the arrow 2 as shown in Fig. 2. 120

The hydrocarbon vapours are thus raised in the retort to a temperature between  $520^{\circ}$  and  $530^{\circ}$  C., after having been subjected to a molecular transformation due to the action of the catalysts which, as is well known, have more or less marked affinities for carbon and hydrogen, and effect at one or another favourable temperature, a displace- 130

ment of the atoms of one or the other of these two substances, which results in a mixture of compounds having physical properties (viscosity, ignition point, density etc.)

5 which are quite different from those of the original hydrocarbons. In short, hydrocarbons are produced in which the atomic groups are less and less condensed.

The vapours leaving the retort as shown 10 by the arrow 3 are brought into an expansion and cooling apparatus B consisting of two truncated cone shaped sheet metal pieces constituting a double casing, and of an inner cylindrical body e connected by tubes 15 f and f' with the annular chamber formed by the double casing.

The hydrocarbon vapours circulate through the annular part of the truncated cone d according to the arrows 4. Water, 20 is thus maintained in ebullition and at a pressure of 10 to 12 kilogrammes in the annular space between d and d' and in the cylindrical body e, so that a constant temperature between 200 and 220° C. will prevail in 25 the part wherein the hydrocarbon vapours circulate.

In this expansion and cooling apparatus, hydrocarbon vapours are subjected to two contrary actions; on the one hand the molecular expansion produced by the change in 30 the volume occupied by the vapours, and on the other hand the contraction due to the abrupt cooling.

The hydrocarbon vapours are discharged, 35 at the lower part of the expansion and cooling apparatus B, into a space whose diameter is 10 or 15 times that of the orifice leading thereto, and hence the molecules composing these vapours will "widen out", so to speak, 40 and will hence become more voluminous; so that a molecular expansion is in fact produced.

Moreover these discharged vapours are at a temperature of 530° C. and since the water 45 boiling under pressure is maintained in the apparatus between 210° C. and 220° C., these same hydrocarbon vapours will undergo a very abrupt cooling, and their temperature falls at once from 530° to 250° C., and a 50 molecular contraction necessarily takes place.

These simultaneous and contrary actions result in a great disturbance in the molecules, and the metallic fragments disposed on the 55 discs g will facilitate certain molecular rearrangements between the unduly heavy hydrocarbon vapours and the very light vapours, or even gases, and which, when properly associated together, will produce a light 60 fuel analogous to gasoline, thus completing the physico-chemical reactions which commenced in the retort.

Furthermore, certain light hydrocarbons of an unstable nature, formed in the retort, 65 are definitely fixed in the state of stable com-

bination by the expansion and contraction to which they are subjected.

But the oil has not been entirely decomposed into lighter hydrocarbons, and a part of the same remains in its original state of 70 more or less heavy hydrocarbons; the fraction distilling above 240°-250° C. is condensed and falls to the bottom of the expansion apparatus B whence it is evacuated through a pipe h and returns into the boiler v after being mixed, if necessary, with a portion of petroleum not yet treated supplied by a pipe i, and which it will thus heat to a temperature of about 200° C. in order to prevent calefaction of said fresh petroleum 80 in the boiler.

The hydrocarbons remaining in the state of vapour below 250° C. and composed for the major part, of the above said light products which have just been manufactured, are led (arrows 5) into a second expansion and cooling apparatus C of a like construction, but wherein the pressure of the boiling water is maintained at only 3 kilogrammes, i. e. at 85 a temperature of about 135° C. 90

The same physical and catalytic actions are repeated in said second apparatus C., but now only upon hydrocarbons distilling below 250° C. and whereof the major part has already undergone a total transformation or a partial doubling; so that the catalytic work in this second expansion and cooling apparatus is simplified, and a definite stability takes place within the mass of the hydrocarbons wherein the atoms of carbon and hydrogen, or their groups of hydrocarbon molecules, were not yet in a perfectly fixed state. 95

Those of said hydrocarbons which distil above 180° C. will condense and fall to the bottom of the second expansion apparatus C, whence they are evacuated through a pipe 100 m and are led to the bottom of the first expansion and cooling apparatus B. 105

The hydrocarbons which are not condensed in the second expansion and cooling apparatus C proceed according to the arrows 6 into an ordinary refrigerator r with cold water or air circulation, in which is condensed the new liquid fuel according to the invention, and whose principal characteristic features have been above explained. Said product is then collected through the cock or valve n in one of the vessels in common use for the storage or transportation of petroliums, 110 gasolines or other volatile liquid products. 115

Having now described my invention what I claim as new and desire to secure by Letters Patent is:

A motor fuel consisting of a stable mixture of more than 50 per cent of unsaturated hydrocarbons with saturated hydrocarbons, the fraction of said mixture distilling between 80° C. and 90° C. remaining substantially free from nitrobenzene when treated 120 125 130

with nitric acid, and the percentage composition of said hydrocarbon mixture being substantially by weight 88 to 89 parts of carbon and 12 to 11 parts of hydrogen.

**5** In testimony whereof I have signed my name to this specification.

**ADOLPHE ANTOINE FRANÇOIS MARIUS SEIGLE.**

**10****15****20****25****30****35****40****45****50****55****60****65**